

Patented Aug. 18, 1925.

## UNITED STATES PATENT OFFICE.

JOSEF PELZER, OF MUNICH, GERMANY.

## PROCESS FOR SIZING PAPER IN THE PULP.

No Drawing.

Application filed June 1, 1923. Serial No. 842,860.

*To all whom it may concern:*

Be it known that I, JOSEF PELZER, a citizen of the German Republic, residing at Munich, Germany, have invented new and useful Improvements in a Process for Sizing Paper in the Pulp, for which I have filed an application in Germany June 6, 1922, No. 371,380, and of which the following is a specification.

0 My invention relates to paper making, and has particular reference to a method of sizing paper in the pulp.

The object of my invention is to provide a method of sizing which may be reliably controlled whereby an increase in efficiency and economy of material is accordingly effected.

It is well known that for sizing paper in the pulp, a watery alkaline solution of 10 rosin containing 90 to 95% of rosin acids may be used, which is added to the paper pulp in the pulp-engine. Then an acid solution of aluminum sulphate is added, whereby, according to universal opinion, the 15 rosin is precipitated throughout the paper in an extremely finely divided state. Since rosin has no affinity for ink or similar watery solutions, the spreading of the ink along the paper fibres is prevented and the 20 paper is thus made suitable for writing purposes.

According to Illig, the inventor of the rosin-sizing process, whose free rosin theory was subsequently supported experimentally 15 by Wurster (Dingler's Polytechnisches Journal 1877), the sizing is effected only by the free rosin, and the most important requirement is to bring the rosin or the rosin acids into contact with the fibres in the finest 20 possible divided state. In accordance with this very plausible explanation of the sizing process, use was frequently made of rosin size alleged to contain free rosin, obtained by boiling the rosin with less alkali 25 than is necessary for the formation of the neutral rosin soap, the rosin being considered to be present in the form of an emulsion.

Upon diluting the rosin soap with water 30 before it is introduced into the pulp-engine, more or less turbid liquids are formed according to the alkali content. This turbidity was explained as resulting from free rosin which, in the case of neutral size, was

supposed to have been formed by hydrolysis, 55 and which, in the case of free-rosin sizes, was believed to be due to the free rosin in an emulsive or very finely divided state.

This theory was frequently borne out by 60 practical experience but just as frequently inexplicable failures occurred. In short, it was impossible sufficiently to control the process, and to avoid failure it was customary to add a surplus amount of size.

I have found however that the free rosin 65 acid is not formed simply by the hydrolysis of the rosin soap solution but that, according to the concentration, different quantities of acid salts are produced, and a state of equilibrium is reached between the following reactions:

$$\text{HsNa} + \text{H}_2\text{O} = \text{NaOH} + \text{HsH}$$
 and 
$$4\text{HsNa} + 3\text{H}_2\text{O} = 3\text{NaOH} + \text{HsNa.3HsH}$$

in which Hs represents the anion of the 75 rosin acid. The free rosin formed by hydrolysis is precipitated in the form of large flakes, while only the acid salt results in the finely divided state required for sizing. It is this acid salt which is absorbed by 80 the fibres and then wholly or partly decomposed by the acid action of the aluminum sulphate. Such acid salt as may remain undecomposed has exactly the same 85 effect as free rosin, since the acid salt has even less affinity for water than rosin.

Because of the temporary existence of this acid salt, until now overlooked, the success 90 of the sizing process has heretofore been more or less a matter of accident. In rosin size supposed to contain free rosin, the latter is not contained as an emulsion in the rosin soap, but on the contrary, the size consists of a mixture of neutral and acid salts 95 of rosin acids in varying amounts. By diluting such sizes, there naturally results in the turbid solution a larger percentage of acid salt than in the case of the hydrolysis of a neutral soap by solution. This percentage can be increased in both kinds of 100 sizes by partly saturating the alkali when dissolving the soap.

Summarizing, it may be said that the reliability and success of the sizing process is 105 dependent only upon a correct controlling of the process by a proper choice of concentration during the action of the soap, and by a regulation of the degree of alkaliza-

tion, so that a maximum amount of acid salt is existent during the sizing and precipitation in the pulp-engine, the acid salt alone being effective since it alone is finely enough divided.

What I claim as my invention and desire to secure by Letters Patent is  
The herein-described method of sizing paper in the pulp, which consists in so con-

trolling the concentration and regulating the alkalization during sizing that a maximum of acid salt of the formula



is produced in the solution.

In testimony whereof I hereunto affix my signature.

DR. JOSEF PELZER.